

1

3,199,211

**METHOD OF PRESEASONING GREEN OR PARTIALLY SEASONED WOOD**

Ralph H. Bescher, Pittsburgh, Pa., assignor to Koppers Company, Inc., a corporation of Delaware  
No Drawing. Filed Feb. 16, 1962, Ser. No. 173,774  
6 Claims. (Cl. 34—9.5)

This application is a continuation-in-part of my co-pending application Serial No. 821,661, filed June 22, 1959, and now abandoned.

This invention relates generally to the preservation of wood in a manner to preseason the wood in a fire-proof hazardless process by means of liquefied petroleum gas.

A common practice in the wood preserving industry is to season wood prior to, during or after impregnating the wood with a preservative. A conventional method of seasoning wood has been to air dry the wood, that is, the wood is placed or stored in a lumber yard to await the natural evaporation and evacuation of the water from the wood.

It is well known that green lumber contains water in two different conditions, that is, a portion of the water is free in the wood, whereas the remainder is actually bound in the cellulosic material of the wood and is considered to have saturated the fibers of the wood.

This air drying method of seasoning is primarily used to remove the free water contained in green wood. The green or unseasoned wood that is exposed to the open air but protected from rain will gradually dry out until the greatest portion of the free water has been removed. The normal procedure in the wood preserving industry, after air seasoning is completed, is to place this pre-seasoned wood into a kiln and under high temperatures force as much of the remaining water as possible to evaporate from the wood.

The commonly used method of air seasoning wood has not proven entirely satisfactory because of the excessive costs necessitated by the length of time required to remove the water in this manner, and because of the high inventory of wood which must be kept on hand during the time the seasoning is taking place in the air. Additionally, sapwood material and the heartwood of non-durable species may become infected with decay (storage rot) in the seasoning pile especially during warm, humid weather.

In addition to seasoning lumber, it has been common practice to treat wood chemically, either before the lumber has been dried or after drying has occurred to increase the service life when the wood is to be used under conditions that favor the early deterioration of the wood as by decay, insects and other destructive agencies. This treatment of wood is generally carried out by forcing preservative chemicals into the wood by pressure. Conventionally, this treatment involves subjecting the wood to a predetermined air pressure (super-atmospheric or sub-atmospheric) and without releasing this pressure, introducing a bath of a preservative onto the wood, then increasing the pressure and usually elevating the temperature of the preservative nearly to the boiling point of water and maintaining this elevated pressure for an interval of time to obtain the desired injection of the preservative in the wood. Thereafter, the bath of preservative is removed from the wood and the wood is sub-

2

jected to sub-atmospheric pressure whereby excess preservative solution is removed from the wood.

The pressure treatment of wood is conventionally denoted as a full-cell or an empty-cell process depending upon the extent of retention of the preservative in the wood. These two processes differ mainly in the initial treating steps. The wood is subjected to sub-atmospheric pressure in the full-cell process so as to empty the cells of air before the wood is subjected to the bath of preservative, and the wood is placed under super-atmospheric air pressure in the empty-cell process to force a considerable amount of air into the cells of the wood before subjecting the wood to a bath of preservative so that when the pressure is released, the air in the cells will eject some of the preservative from the cells.

Conventionally, an aqueous or an oil solution of a preservative is used as the bath. The aqueous or oil solvent places the preservative in a form that will penetrate the cells of the wood. If the wood to be impregnated is green, that is, it has not been air seasoned, a great amount of water will be present. If the cells of the wood contain this great amount of water, it follows that in attempting to impregnate a preservative solution into the wood, the water already contained therein will resist to some extent the penetration of the preservative. As a result, the efficiency of the impregnation process is reduced. Additionally, the presence of the water is undesirable after the preservative is in the wood. The use of water as a carrier for the preservative will increase the amount of water left in the wood and thus requires that the wood be dried subsequent to the impregnation with the preservative. The subsequent drying, of course, requires extra heat and time and is somewhat difficult as the wood cell normally includes water. The moisture content of thoroughly seasoned wood is, for example, within the range of 6 to 15 percent of the dry weight of the wood. Also, the wetting during impregnation and the subsequent drying tends to cause checking of the wood and an undesirable raising of the grain.

The air drying method for seasoning wood hereinabove discussed has included a slow evaporation of the water while the wood is standing in the air for long periods of time. This drying period may extend for from 3 months to three years depending on the particular species of wood being dried.

The principal object of this invention is to obtain an improved process for preseasong green or partially seasoned lumber to obtain a product which (a) does not require an air seasoning period, (b) need not be kept in inventory for any length of time prior to kiln drying or impregnation with a preservative, (c) has had the free water removed within a 24 hour period, (d) is not subjected to excessive heat, (e) is not damaged by treatment, and (f) has not been changed in size.

It has now been found, in accordance with this invention, that wood may be readily preseasonged (free water removed) by subjecting the wood to treatment with an aliphatic hydrocarbon which (a) boils below the boiling point of water at ambient atmospheric pressure, but (b) readily liquefies at ambient atmospheric temperature when placed under elevated pressure.

In the process of this invention, the wood is subjected to a predetermined pressure and then without change in pressure is subjected to an aliphatic hydrocarbon so that the pressure is increased to inject the hydrocarbon into

the wood and thereafter the hydrocarbon evaporates from the wood.

Using the process hereinabove described, it is possible to remove the free water contained in green or in partially seasoned wood by the mechanical action of the hydrocarbon when it leaves the wood.

The novel process of this invention is applicable to all commercial species of wood. In fact, it has been found that the process of this invention is applicable to pre-seasoning refractory species (those species of wood which resist penetration more than the conventional species).

The above defined method of preseasonging lumber is economically and conveniently effective in apparatus commonly used for pressure treatment of lumber. In this respect, it is a novel method of removing the free water from green lumber in that while other processes of impregnation will normally leave water in the green lumber during pressure impregnation or will attempt to evaporate the water with excessive temperatures, the novel process of this invention is a mechanical process wherein the water is literally kicked out of the wood by the expanding aliphatic hydrocarbon gas. As a result of the novel mechanical removal of water, there is no checking of the wood nor undesirable time consuming, waiting period prior to kiln drying or impregnating the wood with a preservative.

The novel process of this invention will remove at least 50% of the free water contained in green or partially seasoned wood. The amount of water removed during the processing will, of course, depend upon the species of wood being treated. For any species, however, at least 50% of the free water is removed. The removal of this amount of water from wood in the very short period of time (less than 24 hours) is a totally unexpected, unusual and novel result. Since it has heretofore been common to air season for up to three years certain species of lumber, the removal of at least 50% of the free water from wood according to the process of this invention makes this invention an extremely practical and time saving method for preseasonging green or partially seasoned wood.

Suitable hydrocarbons for use in accordance with this invention include, for example: liquefied petroleum gas, butane, isobutane, propane, etc. The boiling point and heat of vaporization of these hydrocarbons is such that the temperature and heat of the wood itself is sufficient so that, when the wood is removed from contact with the bath and the pressure lowered, this heat stored in the wood will vaporize the solvent remaining on and in the wood.

Accordingly, the process is desirably carried out at temperatures and pressures at which the solvent will be self-evaporating from the wood when the bath is removed from the wood. These hydrocarbons have vapor pressures such that the wood can be heated from 150 to 200° F. without developing excessive pressure. The application of high pressure to the wood has a tendency to damage the wood by crushing the cells of the wood. In addition, temperatures higher than 200° F. tend to weaken the cell structure of the wood so that the wood becomes more susceptible to crushing under pressure.

The processing of wood in accordance with this invention, wherein wood is preseasonged in a low boiling hydrocarbon has manifold advantages. The treated wood is clean; there is a decrease in weight of the wood; since the hydrocarbon has no affinity for wood, as does water, and since the vapor pressure of the hydrocarbon is greater than the final pressure in the treating chamber, the hydrocarbon readily escapes from the wood. Thus, air storage is not required. The hydrocarbon itself serves as an instrument for removing the residual free water from the wood, i.e., at the conclusion of the pressure phase, the rapidly expanding solvent gases expel the free water from the wood. The wood treated in accordance with this invention leaves the bath substantially dimensionally unchanged. Wood treated in accordance with this invention is odorless and has a non-oily surface, an advantage, of course, if the wood is to be painted.

The empty cell process is advantageously used to afford a fireproof, hazardless procedure with this process, as the high vapor pressure of the solvent aids in the ejection of the hydrocarbon from the cells at the end of the pressure treating step of the process, thereby reducing the quantity of hydrocarbon which must be evaporated from the wood. The gas used for impregnating the cells prior to their impregnation with the solvent and preservative may be air, but preferably is nitrogen, carbon dioxide, or other inert non-condensable gases since the hydrocarbons are flammable. The empty cell process may be used with complete safety and freedom from fire or other hazardous conditions even though the vapor pressure characteristics of the solvent lends itself to full cell process.

The invention will be illustrated further by comparison of the empty cell process in Example II with the full cell processes in Examples I and III in the following examples.

#### EXAMPLE I

Green timbers of southern pine are placed in a closed cylinder and a vacuum of 25 inches of mercury is maintained on the cylinder for one half hour. Then, without admitting air, the cylinder is filled with liquid butane. The cylinder is then heated until the pressure in the cylinder increases to 125-200 pounds per square inch gauge. During the heating period, additional solution is pumped into the wood and to maintain the pressure at 125-200 pounds per square inch gauge pressure, and these pressures and temperatures are maintained on the wood for about two hours. Then, the hydrocarbon solution is removed from the cylinder and the cylinder subjected to a vacuum of 25 inches of mercury for an hour. Thereafter, the wood is removed from the cylinder. The wood is substantially dry, clean and odorless.

#### EXAMPLE II

Green timbers of southern pine are placed in a closed container and air in amounts beyond the explosive limits, or nitrogen or carbon dioxide, is injected into the container until the pressure in the container reaches 50 pounds per square inch gauge. Thereafter, butane is forced into the container and air is withdrawn from the container at a rate to maintain a constant pressure of 50 pounds per square inch gauge in the container. After the solution fills the container, the pressure is increased to 200 pounds per square inch gauge by raising the temperature, this pressure maintained for two hours, and then released. As soon as this pressure is released, the compressed gas in the wood expands and forces the hydrocarbon from the wood to a considerable extent. The hydrocarbon is drained from the cylinder and the wood subjected to a vacuum of 25 inches of mercury for a period of an hour, during which time the heat in the wood evaporates the solvent remaining.

#### EXAMPLE III

Green southern pine is placed in a closed container and subjected to steam at a pressure of 15 pounds per square inch gauge for six hours. The steam is released and the cylinder evacuated for a period of two hours. Thereafter, butane is pumped into the cylinder, and after the butane fills the cylinder, the butane is heated to increase the pressure to about 200 pounds per square inch gauge and this pressure maintained for two hours. The pressure is then released and the wood subjected to a vacuum of 25 inches of mercury for a period of thirty minutes. The wood presents a product that has been partially dried in less than 10 hours.

#### EXAMPLE IV

Hard maple 1" by 3" by 4' is placed in a closed container and subjected to steam at a pressure of 15 pounds per square inch gauge for 6 hours. The steam is released and the container evacuated for a period of 2 hours. Thereafter, isobutane is pumped into the container and

after the isobutane fills the container, the isobutane is heated to increase the pressure to about 200 pounds per square inch gauge and this pressure maintained for 2 hours. The pressure is then released and then following this release of pressure, another pressure period of approximately 2 hours is again applied to the maple in the cylinder. Then pressure of the second pressure period is released and the wood is subjected to a vacuum of 25 inches of mercury for a period of 30 minutes. The wood is then removed from the cylinder and the moisture content is measured. For these particular species of wood, the moisture content was reduced from 57% to 36%.

#### EXAMPLE V

Four stump green southern yellow pine poles were season-treated with liquefied petroleum gas. A total of 7 hours pressure was used followed by a 2 hour final vacuum. The poles had an average butt diameter of 10 in. and were 36 ft. long. Before treatment, these poles weighed 63.4 lbs./cu. ft. and following treatment they weighed 49.8 lbs./cu. ft. In other words, during the treatment 13.6 lbs. of water was removed from each cubic foot of wood.

#### EXAMPLE VI

Stump green southern yellow pine poles were season-treated with isobutane. A total of 7 hours pressure was used followed by a 2 hour final vacuum. The poles had average butt diameters of 10 in. and were 36 ft. long. During treatment, the weight per cubic foot of these poles was reduced from 59.6 to 44.0 lbs./cu. ft.

#### EXAMPLE VII

Stump green southern yellow pine poles were treated and seasoned with isobutane. A total of 7 hours pressure was used followed by a 2 hour final vacuum. These poles had an average butt diameter of 10" and were 36' long. The average moisture content of the outer 1 in. of these poles was 65% before treatment and 33% after treatment. Approximately 11.7 lbs. of water was removed per cubic foot of wood.

As further verification of the ability of this process to remove the free water contained in green or partially seasoned lumber, several other specimens of southern yellow pine and redwood lumber were subjected to treatment with liquefied petroleum gases and tested for moisture content before and after treatment. The results of the treatment of the southern yellow pine poles are shown below in Table I.

Table I  
SEASONING DATA ON SOUTHERN YELLOW PINE POLES

| Pole No. | Dimensions       |                 |                  | Moisture Content (Percent) |    |              |    | Wt. Loss, lb./cu. ft. |
|----------|------------------|-----------------|------------------|----------------------------|----|--------------|----|-----------------------|
|          |                  |                 |                  | Outer 1"                   |    | 1" to 2 1/4" |    |                       |
|          | Before Treatment | After Treatment | Before Treatment | After Treatment            |    |              |    |                       |
| 1.....   | 10.3             | 35.7            | 20.6             | 143                        | 42 | 82           | 51 | 13.6                  |
| 2.....   | 10.2             | 35.5            | 20.3             | 92                         | 57 | 103          | 65 | 60                    |
| 3.....   | 9.7              | 35.9            | 18.4             | 58                         | 39 | 86           | 47 | 55                    |
| 4.....   | 11.4             | 35.8            | 26.3             | 108                        | 52 | 91           | 65 | 55                    |
| 5.....   | 10.9             | 35.8            | 22.9             | 110                        | 51 | 118          | 60 | 55                    |
| 6.....   | 10.4             | 35.6            | 20.8             | 111                        | 49 | 110          | 48 | 55                    |
| 7.....   | 10.8             | 35.0            | 22.1             | 124                        | 35 | 91           | 36 | 55                    |
| 8.....   | 9.6              | 35.5            | 17.9             | 91                         | 33 | 108          | 46 | 55                    |
| 9.....   | 10.8             | 35.5            | 22.8             | 61                         | 33 | 79           | 30 | 55                    |

In the production of redwood lumber, the lumber is generally classified as heavy and medium in moisture content. The normal method of seasoning material of this classification has been to first air season the lumber to approximately 65% moisture content for about 9 to 18 months and then kiln dry it to a final moisture content of about 10%. Using the process of this invention, the moisture level of heavy or medium segregation can be

immediately reduced to about 65% in less than 24 hours, obviating the use or the need of any prolonged air seasoning. Table II shows the results of 21 specimens of redwood lumber which were preseasoned according to this invention and then measured for moisture content after seasoning.

Table II  
SEASONING DATA ON REDWOOD LUMBER  
[Dimensions 2 x 6 x 8]

| Board No. | Moisture Content (Percent) |                 | Wt. Loss, lb./cu. ft. | Moisture Content Reduction (Percent) |
|-----------|----------------------------|-----------------|-----------------------|--------------------------------------|
|           | Before Treatment           | After Treatment |                       |                                      |
| 1.....    | 162                        | 75              | -22.4                 | 87                                   |
| 2.....    | 150                        | 48              | -29.0                 | 105                                  |
| 3.....    | 150                        | 45              | -29.4                 | 105                                  |
| 4.....    | 114                        | 60              | -10.0                 | 84                                   |
| 5.....    | 114                        | 63              | -13.2                 | 51                                   |
| 6.....    | 131                        | 61              | -19.0                 | 70                                   |
| 7.....    | 131                        | 61              | -18.5                 | 70                                   |
| 8.....    | 172                        | 69              | -27.0                 | 103                                  |
| 9.....    | 172                        | 74              | -25.8                 | 98                                   |
| 10.....   | 172                        | 64              | -26.7                 | 108                                  |

The foregoing has presented a novel process for the safe preseasoning of wood with a hydrocarbon selected from the class consisting of aliphatic hydrocarbons which may be liquefied at ambient temperatures by subjecting the gases to an elevated pressure. The hydrocarbon is self-evaporating so that the wood needs no drying period for the removal of hydrocarbon. The solvent, in addition to self-evaporation from the wood, creates a mechanical force which removes the free water contained in green or partially seasoned lumber and thus exerts a preseasoning effect upon the wood.

What is claimed is:

1. A method of rapidly preseasoning green and partially seasoned wood which comprises the steps of:  
subjecting said wood to a predetermined pressure with inert non-condensable gas so as to impregnate the wood with said gas, and thereafter without changing the pressure,  
subjecting said wood to an aliphatic hydrocarbon which boils below the boiling point of water but which can be liquefied at ambient temperature conditions at pressure above atmospheric pressure and which is a liquefied petroleum gas selected from the group consisting of butane, isobutane, propane and isopropane, subjecting said wood and hydrocarbon to increased pressure whereby the hydrocarbon penetrates said wood as a liquid, and  
thereafter releasing the pressure, thereby expanding the non-condensable gas and evaporating the hydrocarbon and thus expelling the free water and removing the hydrocarbon from the wood.
2. A method of quickly preseasoning green and partially seasoned wood by removing the free water therefrom which comprises the steps of:  
subjecting said wood to a predetermined pressure with inert non-condensable gas so as to impregnate the wood with said gas,  
thereafter without changing the pressure, subjecting said wood to an aliphatic hydrocarbon which boils below the boiling point of water but which can be liquefied at ambient temperature conditions at pressures above atmospheric pressure and which is a liquefied petroleum gas selected from the group consisting of butane, isobutane, propane and isopropane, subjecting said wood and hydrocarbon to increased pressure whereby the hydrocarbon penetrates said wood as a liquid, and  
thereafter evaporating the hydrocarbon from the wood due to the stored heat in the wood, whereby the hydrocarbon vapors leave the wood and expel water.

from the wood, and whereby said preseasonging occurs in less than a 24-hour period.

3. A process for preseasonging green or partially sea-  
5 soned lumber to obtain a product which does not re-  
quire an air seasoning period, need not be kept in in-  
ventory for a length of time prior to kiln drying or im-  
pregnation with a preservative, and has at least 50% of  
the free water removed within a 24-hour period, the  
process:

subjecting said wood to an elevated pressure with an  
inert non-condensable gas so as to impregnate the  
wood with said gas,  
thereafter without changing the pressure, subjecting said  
wood to a lower aliphatic hydrocarbon which boils  
below the boiling point of water but which can be  
liquefied at ambient temperature conditions at pres-  
15 sures above atmospheric pressure and which is a  
liquefied petroleum gas selected from the group con-  
sisting of butane, isobutane, propane and isopropane,  
elevating the temperature of the hydrocarbon and the  
20 wood to a temperature of from 150 to 200° F. while  
maintaining the hydrocarbon as a liquid whereby the  
pressure increases and the liquid hydrocarbon pen-  
etrates said wood, and  
thereafter releasing the pressure to expand the non-  
25 condensable gas and to vaporize the hydrocarbon  
whereby the free water is expelled and hydrocarbon  
is removed from the wood to provide a preseasoned  
wood which is dry in that at least 50% of the free  
water has been removed therefrom and which has a  
30 non-oily surface.

4. A process of rapidly preseasonging green and partially  
35 seaoned wood which comprises:

impregnating wood with a liquid hydrocarbon which  
is a liquefied petroleum gas selected from the group  
consisting of butane, isobutane, propane and isopro-  
pane under superatmospheric pressure, and  
releasing said pressure so that said hydrocarbon auto-  
35 genously vaporizes and the vapors expel the free  
water in liquid form from the wood.

5. A process of rapidly preseasonging green and partial-  
ly seaoned wood which comprises:

injecting a liquid hydrocarbon which is a liquefied

petroleum gas selected from the group consisting  
of butane, isobutane, propane and isopropane into  
wood,

heating said wood and hydrocarbon under pressure,  
and  
releasing said pressure to vaporize said hydrocarbon  
so that the vapors expel the free water as a liquid  
from the wood.

6. A method of preseasonging green and partially sea-  
5 soned wood which comprises the steps of  
subjecting said wood to a liquid aliphatic hydrocarbon  
which is a liquefied petroleum gas selected from the  
group consisting of butane, isobutane, propane and  
isopropane,  
subjecting said wood and hydrocarbon to increased  
pressure whereby the hydrocarbon is injected into  
said wood as a liquid, and  
thereafter releasing the pressure and evaporating the  
hydrocarbon and thus expelling the free water as a  
liquid by the hydrocarbon vapors and removing the  
hydrocarbon from the wood.

#### References Cited by the Examiner

##### UNITED STATES PATENTS

|           |       |            |          |
|-----------|-------|------------|----------|
| 1,023,745 | 4/12  | Marr       | 117-59   |
| 1,760,444 | 5/30  | Secord     | 34-9.5 X |
| 1,967,990 | 7/34  | Edwards    | 34-9.5 X |
| 2,152,665 | 4/39  | Rosenthal  | 34-37 X  |
| 2,507,190 | 5/50  | Barksdale  | 34-9.5   |
| 2,860,070 | 11/58 | McDonald   |          |
| 2,892,261 | 6/59  | Hutchinson | 34-9.5   |

##### OTHER REFERENCES

Encyclopedia of Chemical Technology, vol. 7, pages  
632 and 639, 1951 Ed., The Interscience Encyclopedia  
Inc., N.Y.

40 Encyclopedia of Chemical Technology, Vol. 10, 1953,  
page 138, The Interscience Encyclopedia Inc., New York.

NORMAN YUDKOFF, Primary Examiner.

UNITED STATES PATENT OFFICE  
CERTIFICATE OF CORRECTION

Patent No. 3,199,211

August 10, 196

Ralph H. Bescher

It is hereby certified that error appears in the above numbered patent requiring correction and that the said Letters Patent should read as corrected below.

Column 4, line 27, after "the", first occurrence, insert -- cylinder to replace the material forced into the --; lines 50 and 51, for "subpected to a vaccum" read -- subjected to a vacuum --; column 6, line 47, for "pressure", first occurrence, read -- pressures --.

Signed and sealed this 29th day of March 1966.

(SEAL)

Attest:

ERNEST W. SWIDER

Attesting Officer

EDWARD J. BRENNER

Commissioner of Patents